

# UNITED STATES PATENT OFFICE.

WILLIAM HALES TURNER, OF TUNSTALL, COUNTY OF STAFFORD, ENGLAND.

## METHOD OF PRINTING AND DECORATING CHINA.

SPECIFICATION forming part of Letters Patent No. 391,346, dated October 16, 1888.

Application filed February 5, 1887. Serial No. 226,711. (No specimens.) Patented in England January 4, 1887, No. 120.

*To all whom it may concern:*

Be it known that I, WILLIAM HALES TURNER, a subject of the Queen of Great Britain, residing at Tunstall, in the county of Stafford, 5 England, earthenware-manufacturer, have invented new and useful Improvements in the Printing or Decorating of Earthenware, China, and the like, and in the preparation or manufacture of materials therefor, (for which I have obtained a patent in Great Britain, No. 120, 10 dated January 4, 1887,) of which the following is a specification.

This invention relates to improvements in the preparation of paper with transfer-designs 15 thereon for the decoration of pottery-ware, and comprises novel features in the composition of the size for the paper, in the preparation of the coloring materials, and in the mode of applying the same. The object thereof is to enable the patterns or designs to be printed rapidly in mineral colors, most of which contain a great proportion of metallic oxide of a very abrasive character, which, under ordinary circumstances, rapidly wears away both the printing-surface 20 or block and the doctors or scrapers. In order to print successfully in mineral colors, and prevent undue wear of the parts in contact therewith, it is necessary that such parts, and also the colors themselves, should be heated to an extent not hitherto practiced in the art of pottery-printing. It is impossible, in fact, to increase the temperature too highly, so long as 25 the colors are not burned.

In order to render the paper suitable for the 30 reception of colors and of a quality that will allow it to part readily with the same when transferred to the china or earthenware, it is "sized" with the following preparation: To one gallon of water I add two pounds of soda, 35 and boil until the soda is dissolved. Half a pound of white lead is then added, and, lastly, a pint of linseed-oil, and the boiling continued until a thorough mixture of the ingredients is effected. The paper may be sized in the usual 40 manner, either at the mill or during its passage through the printing-machine; but the former is preferred, as the size is then firmly set before being used. The effect of the size is to destroy the fiber of the paper and fill up 45 the pores thereof, so as to prevent any absorption

of the coloring-matter and render the paper easily friable when moistened.

The coloring materials are prepared as follows: To one gallon of boiling oil I add one pound of tar, the mixture being allowed to boil for half an hour, when I add a quarter of a pound of white lead, allowing the boiling to continue for three or four hours, when a small quantity of sugar—say, half an ounce—is added, and the boiling continued for another hour, at the expiration of which time it will have attained the required consistency or adhesiveness. The mixture is then gradually cooled and stored for future use, becoming, according to present experience, more suitable for use as a vehicle for coloring materials in proportion to the length of time it is kept. The coloring-matter to be mixed with the above vehicle, after being ground as fine as possible and "lawned" or sifted, is highly heated, care being taken not to burn it. The vehicle is then boiled and the heated coloring-matter introduced, and the whole thoroughly mixed or ground together, preferably by hollow heated granite cylinders, until ready for use. 75

In order to derive the full benefit of my invention, it is necessary that the paper and colors at the time of printing should be highly heated—say to about 400° Fahrenheit. A lower temperature will suffice; but under such conditions it will be necessary to allow the paper to remain longer in contact with the printing block or cylinder, whereby the rate of production will be diminished. 80

I do not confine myself to the proportions of the various ingredients herein given, nor to the exact time required, or mode of procedure, although I have found such to be satisfactory.

The paper prepared in accordance with my method with ornamental designs thereon is employed in the usual manner by applying it to the articles to be decorated and transferring the designs thereto by pressure with or without the application of heat and thereafter removing the paper by saturating it with water. 90

What I claim as my invention is—

1. The process of preparing transfer-paper for decorating china, consisting, first, in charging the paper with size, substantially such as

specified herein, to fill its pores, then printing the design in mineral colors, combined with oil, tar, white lead, and sugar, in the presence of pressure and heat.

5 2. The process of preparing paper with ornamental designs in color for transference to china, consisting of the following steps: first, charging the paper with a size composed of soda, white lead, and oil; second, applying to the sized paper in the presence of heat and

pressure a metallic coloring-matter, combined with oil, tar, white lead, and sugar.

In testimony whereof I have hereto set my hand in the presence of the two subscribing witnesses.

WILLIAM HALE TURNER.

Witnesses:

ARTHUR V. LLEWELLYN,

SAML. DAVIES,

*Both Solicitors, Tunstall, England.*